

## UNITED STATES PATENT OFFICE

JEAN JULES LAMBRECHT, OF NIEPPE, FRANCE

## PROCESS FOR THE MANUFACTURE OF VEGETABLE WOOL

No Drawing. Application filed May 31, 1929, Serial No. 367,637, and in France June 9, 1928.

This invention relates to a new application of the treatment of vegetable fibers disclosed in the application Serial No. 290,049 of July 2nd, 1928.

5 Said new application not only prevents the treated fibers from putrefaction but lends them sufficient strength to resist subsequently a treatment with acids or soda for the purpose of giving them the appearance of animal wool.

The process disclosed in above mentioned patent application consists essentially in causing the penetration, into any vegetable fibers, of a fat (mineral oil or any other fatty matter) introduced at high temperature in a 15 boiling bath of saponified fats, specially containing mineral oils.

According to this invention, above means applied in a new way are combined with various treatments which give the textile fibers 20 the appearance of animal wool.

As an example of the manner this invention can be carried out, a succession of treatments of vegetable fibers will be described hereinafter.

The fibers are first treated mechanically for the purpose of rendering them flexible and in order to separate the small pellicles and part of the gum which may adhere to said 30 fibers.

After this mechanical treatment has been achieved, the flexible fibers are introduced into a suitable vat in which is circulating a hot bath containing, for one liter of water,

35 3 grams of oleic acid,  
2 grams of mineral oil,  
1 gram of 36° Bé. soda lye,  
1 gram of sodium carbonate.

40 This hot bath circulates at a great speed in said vat which contains the vegetable fibers, this speed being approximately one meter per second. The duration of the operation may last from one and a half to four hours according to the kind of fibers.

45 The mineral oil, which is saponified or emulsified by the presence of the base, lubricates the fibers and protects them against the corrosive and destructive action of the subsequent treatment described hereinafter. This

lubrication permits the retention in the fibers of the whole of the cellulose they contain.

The fibers thus lubricated are thereupon plunged into a cold bath of caustic soda of 10 to 24° Bé., the contents of the bath in soda 55 being subject to variations according to the kind of fibers treated. This immersion is continued during a time which may vary, also according to the kind of fibers, from fifteen minutes to three hours. As in the previous bath this bath of caustic soda will pass rapidly through the vat in which the fibers are maintained.

After this treatment the fibers are rinsed and submitted to the action of baths which 60 circulate rapidly and which are suitably acidified in order to neutralize the excess of caustic soda which may be contained in the fibers.

The fibers are then submitted to the bleaching action of a bath of sodium hypochlorite containing twenty five grams per liter or to any equivalent treatment.

The fibers are then rinsed and finally submitted to a softening bath containing a neutral soap and sodium monosulfide; these compounds may be contained in the bath in the ratio of 10 grams of soap and one gram of sodium monosulfide for a liter of water. The duration of the immersion in this bath varies 75 from half an hour to two hours according to the kind of fibers.

Finally the fibers are wrung and dried by the means usually used for mineral wool.

A vegetable wool with the appearance of 80 animal wool is thus obtained.

It is to be understood, as said before, that the proportions of materials contained in the various baths to which they are submitted may vary according to the kind of fibers to 90 which this process applies. It is also to be understood that, without altering the scope of the invention, the kind of the materials entering into the composition of the baths may be altered in some cases as long as the properties of said baths do not suffer thereby.

What I claim is:—

Process of treatment of vegetable fibers, to give them the properties of animal wool, comprising a mechanical treatment for the 100

separation of small pellicles and part of the  
adhering gums, a protective lubricating treat-  
ment of the fibers with a hot saponifying  
bath, a treatment with a rapidly circulating  
5 cold caustic lye, a neutralization by immer-  
sion in an acidulated and rapidly circulating  
bath, the bleaching of the fibers, the rinsing  
of the fibers, the treatment by a softening bath  
containing neutral soap and sodium monosul-  
10 fide and the wringing and drying of the fibers.

10 In testimony whereof I have signed this  
specification.

**JEAN JULES LAMBRECHT.**

**15**

**20**

**25**

**30**

**35**

**40**

**45**

**50**

**55**

**60**

**65**